# EUROPEAN PATENT SPECIFICATION

(11) **EP 2 540 175 B1**
(45) Date of publication and mention of the grant of the patent: **11.08.2021**
(21) Application number: 10846003.1
(22) Date of filing: 04.11.2010
(51) Int. Cl.: A41D 13/00, D04B 1/18, D04B 1/24, A41D 31/18

(54) **SOFT AND ELASTIC JACKET**
WEICHE UND ELASTISCHE JACKE
VESTE SOUPLE ET ÉLASTIQUE

(30) Priority: 22.02.2010 CN 201010116434
(43) Date of publication of application: 02.01.2013
(73) Proprietor: Toray Fibers & Textile Research Laboratories (China) Co., Ltd., Nantong, Jiangsu 226009 (CN); Toray Industries (HongKong) Ltd. (THK), Harbour City, Kowloon, Hong Kong (CN)
(72) Inventor: NI, Qingmei, Nantong Jiangsu 226009 (CN); LIU, Tongjuan, Nantong Jiangsu 226009 (CN); SHIMIZU, Toshiaki, Otsu Shiga 5208558 (JP); LIU, Juan, Nantong Jiangsu 226009 (CN); MURAKAMI, Masanari, The Gateway, Harbour City, Kowloon Hong Kong (CN)
(74) Representative: Hoefer & Partner Patentanwälte mbB
(86) International application number: PCT/CN2010/078433
(87) International publication number: WO 2011/100881

(56) References cited:
- CN-A- 1 957 125
- CN-A- 101 596 026
- CN-A- 101 596 026
- ES-A1- 2 319 486
- JP-A- 11 200 119
- JP-A- 2005 290 625
- JP-A- 2007 113 147
- JP-A- 2007 182 649
- JP-A- 2007 182 650
- JP-A- 2009 293 145
- US-A1- 2004 016 041
- US-A1- 2005 183 463
- US-A1- 2006 130 532
- None

## Description

### TECHNICAL FIELD

This invention relates to a soft and elastic jacket.

### BACKGROUND ART

People are increasingly paying attention to their own health, daily dietary and life quality, and people doing various kinds of exercises are increasing. Therefore, the people's requirements, especially the performance requirements for the exercise garments, such as sportswear, have been raised accordingly. A soft and elastic jacket integrating comfortableness with sports function becomes a new demand of the people.

At present, for elastic jackets for sports available in the market, the designs thereof are usually focused on how to acquire high elasticity or on how to splice and cut different elastic fabrics such that the elasticity in different portions is different. For certain portions, high elastic fabrics are used to enhance tightening force on the wearer's muscles contacting these portions. For example, Chinese Unexamined Patent Publication CN101351129A discloses an exercise garment which exerts tightening forces on the scapulae and scapulae-surrounding muscle groups, so as to improve the exercise performance in various types of exercise accompanied by rotation of the trunk and movements of the arms. There are also examples in which taping theory is used to exert tightening forces on different parts. For example, Chinese
Unexamined Patent Publication CN 101056551A discloses a compression garment which has the first and second panels of stretchable material joined by a seam. The seam is adapted to correspond to the part of a muscle ridge. The taping theory is used to tighten the muscle ridge and therefore to improve the exercise ability and performances. For example, US Patent Application 2004/0016041 A1 discloses an undershirt worn in an undershirt worn in a state of being substantially in close contact with a surface of an upper body of a wearer includes a main constituent portion made of stretchable materials that include a first-type material, a second-type material, and a third-type material. The three types of materials have different straining and are arranged in different regions, thereby intentionally facilitating a pitching motion and a batting motion. For example, US Patent Application 2006/0130532 A1 discloses a method for making circular-knit elastic fabric comprising spandex and hard yarns, without dry heat setting the fabric as part of the method, which may provide circular knit, elastic, single jersey fabrics that, when collected by folding (plaiting), do not crease to the same extent as similar circular knit single jersey fabrics produced by other methods, thereby increasing a yield for cutting and sewing the fabric into garments. For example, ES Patent Application 2319486 discloses a two-component t-shirt particularly intended for the practice of outdoor racquet sports in cold weather, which comprises a body, two sleeves and a neck and is relatively tight. The elastic fabrics used in these prior art technologies are high elasticity fabrics which exert high tightening forces on human body. For peoples like professional athletes with well developed muscles, their sports performances can be improved by wearing these compression garments. However, for ordinary sports enthusiasts, they may easily feel tired and discomfort, because these compression jackets may tighten the enthusiast's muscles too strong to a too tight state when worn, and may excessively increase burden on the muscles and even the hearts when worn for a long time due to the enthusiasts doing not have hard muscles like professional athletes.

### DISCLOSURE OF THE INVENTION

The purpose of the present invention is to provide a soft and elastic jacket.

The technical solution of the present invention is defined in the appended claims and is as follows:

A soft and elastic jacket being composed of an elastic weft knitted fabric, wherein the elastic weft knitted fabric comprises 5∼15% weight of elastic yarns and the rest of non-elastic yarns knitted with each other, wherein the elastic weft knitted fabric covers no less than 70 percent of the circumference of a body part of the soft and elastic jacket when the soft and elastic jacket is in a motionless state without being worn, and the elastic weft knitted fabric has a tightness index of not greater than 0.8 and a recovery stress of 0.3∼1.3 N at an elongation range of 30∼80%, wherein the tightness index is measured according to a method specified in JIS L-1096:1999, and the recovery stress is measured according to a method specified in JIS L-1096:1999.

The term "tightness index" referred to here means a degree of compression provided by clothing to a human body. It is measured with an IT-DRS stretching fatigue testing machine from INTEC Company of Japan according to the
method specified in JIS L-1096:1999, which was published on April 20, 1999. Sample specimens of 10 cm×15 cm in size are taken separately in both the warp and weft directions. The sample specimens are pulled at a speed of 30 cm/min to 110% with a clamping interval of 7.6 cm and a width of 2.5 cm, and finally, the values of the stress at 30% and 80% elongations are read, respectively. The tightness index is calculated as follows: $Tightness index = \left(\left(Stress of elastic weft knitted fabric at 80% elongation <N1>-Stress of elastic weft knitted fabric at 30% elongation <N2>\right)/50\right) \times 10 .$

In addition, a method for determining the recovery stress is as follows: a tensile testing machine from A & D
Company of Japan is used for the determination according to the method for determining elongation recovery rate and residual elongation rate specified in JIS L-1096:1999. Specifically, the elastic weft knitted fabric is pulled once until the stress thereof reaches 20 N, under which situation the elastic weft knitted fabric has an elongation greater than 80%, and the values of the recovery stresses at 80% elongation and at 30% elongation are read respectively during a recovery process of the elastic weft knitted fabric after being pulled. The recovery stress has close correlation with the comfort level in actual wearing situation. The less the recovery stress is, the less compression and the more comfortable a wearer feels.

The respiratory quotient is not greater than 1.05, when a person wearing it exercises at an exercise intensity of less than 7 Mets and a body exercise amount of not greater than 25 Mets·hr for an exercise time of less than 6 hrs. The term "exercise intensity" referred to here means a degree of physiological stimulation of human body caused by physical exercise. A quantification method thereof is carried out by using oxygen consumption. The exercise intensity for consumption of one kilocalorie per hour per kilogram of body weight is defined as 1 Met. A body exercise amount is the product of the exercise intensity and an exercise time. Unlike compression garments commercially available for professional athletes, the designers paid specific attention to the characteristics of normal sports enthusiasts when designing the soft and elastic jacket. The sports enthusiasts with a habit of daily exercising at an appropriate amount of exercise are the main object of the designer's study. The appropriate amount of exercise is specified in the present invention as a monthly amount of exercise of 50 to 1000 Mets hr.

The term "respiratory quotient" ("RQ" for short) refers to the ratio of the volume or molar of carbon dioxide
released to the volume or molar of oxygen absorbed in an organism in a specified time, i.e. the ratio of the molecular of CO₂ released to the molecular of O₂ absorbed in respiration. Sugars, fats and proteins have different CO₂ outputs and
O₂ consumptions when oxidized. Therefore, these three substances have different respiratory quotients. The respiratory quotients can be classified as protein respiratory quotients and non-protein respiratory quotients. The protein respiratory quotient can be measured by measuring the amount of urinary nitrogen quantity in a specified time, and then calculating the amount of the protein decomposed in vivo based on the amount of urinary nitrogen, and calculating the O₂ consumption and CO₂ output during the decomposition of the proteins. Thus, the non-protein respiratory quotient, i.e., the respiratory quotient of the sugars and fats, can be calculated by subtracting the O₂ consumption and CO₂ output during the composition of the proteins from the measured total O₂ consumption and total CO₂ output. Since more fats are consumed than sugars are in an exercise, the exercise an exerciser does when the non-protein respiratory quotient is small is called as aerobic exercise, which is healthful. In fact, the amount of the proteins for oxidation is so small, in comparison with those of fats and sugars, it can be negligible. Thus, a mixed respiratory quotient so measured can be reckoned as non-protein respiratory quotient. In other words, the smaller the measured value of the respiratory quotient value is, the higher the degree of aerobic exercise an exerciser does is, and the healthier for the exerciser is.

In actual determination, the oxygen consumption and carbon dioxide output of a sports enthusiasts is measured by using a cardio-pulmonary function tester from JAEGER Company of German, and the body weight of a sports enthusiasts is measured by using a human body precision balance from METTLER Company of Japan. Thus, the exercise intensity and the respiratory quotient can be obtained by using the following equation: $Exercise intensity = Oxygen intake < mL / min > / \left(Sports enthusiast's body weight <kg>\times 3.5 <mL/kg⋅min>\right)$ $Respiratory quotient = Oxygen intake < mL / min > / Carbon dioxide output < mL / min >$

The clothing pressure of the soft and elastic jacket is 0.6 kPa or less in a motionless state, 0.60 kPa or less in a portion between the elbow portion and the wrist portion, 0.33 kPa or less in the chest portion, and 0.40 kPa or less in the back side. The clothing pressure is 2.5 kPa or less in a motion state, and 1.25 kPa or less in a portion between the
elbow portion and the wrist portion, 0.45 kPa or less in the chest portion, and 1.85 kPa or less in the back side. The clothing pressure is measured by using a contact pressure tester, in which the diameter of a bag as used is 20 mm, from AMI Company of Japan. The determination is made simultaneously at three points: chest, back and forearm (a portion between the elbow portion and the wrist portion). The term "a motionless state" refers to a state in which the body is upright and the arms are sagging naturally, and the term "a motion state" refers to a state in which exercises,
such as lateral-raising, front-raising, stretching downwards, elbow flexion, expanding the chest, golf swing, doing hori- zontal push-ups, running, riding bicycle, etc., are done to a certain level over a period of time.

The elastic weft knitted fabric in the present invention is produced by knitting 5∼15% weight of elastic yarns with the redundant rest of non-elastic yarns, and has a basis weight of 140-200 g/m². If the content of the elastic yarns is lower than 5%, the tightness index of the elastic weft knitted fabric will exceed 0.8 and the recovery stress on the body
will also exceed 1.3 N at 30∼80% elongation, or the elastic weft knitted fabric can not be stretched to 30∼ 80%. If the content of the elastic yarns is higher than 15%, the content of the elastic yarns will be too high, such that the tightness index of the elastic weft knitted fabric will exceed 0.8 and the recovery stress on the body will exceed 1.3 N at 30∼80% elongation. In other words, the content of the elastic yarns being too low or too high will cause the wearer too tight and difficult to exercise when wearing the elastic jacket.

The elastic yarns are polyurethane fibers. The non-elastic yarns are modified PET fibers and/or polyamide fibers.

The non-elastic yarns are preferably cationic dyeable PET fibers.

The advantages of the invention are as follows: since the elastic weft knitted fabric of the soft and elastic jacket has an appropriate tightness degree, the elastic jacket can be stretched or recovered freely following stretching or recovery of the body skin caused by the wearer's movement within the range of normal exercise movement. Thus, the elastic jacket can reduce the energy excessively generated by human body for resisting the compression from the jacket. On the other hand, the jacket can timely expand or recover to follow stretching or recovery of the body skin caused by wearer's movement. As compared with the elastic jackets of the same kind, wearer will feel lighter, free of burden when wearing a soft and elastic jacket made of the elastic weft knitted fabric and exercising, and it is possible for a person wearing the elastic jacket to do aerobic exercise which is healthful.

### Mode of Carrying out the Invention

The following examples are provided to give further explanation of the present invention.

### Example 1:

84 dtex /72 filament cationic dyeable PET yarns and 33 dtex polyurethane yarns were used in a proportion of
88 to 12 to produce a circular plain knit fabric with a gram weight of 175 g/m². A compression garment of size L using the knit fabric for 100% body circumference was finally made after the treatments of refining, dyeing, and forming. The weft knitted fabric was measured to have a maximal tightness index of 0.7 and a maximal recovery stress of 1.2 N at 30∼80% elongation. A male subject having a body height of 173 cm, a body weight of 72 kg and monthly exercising at an amount of 120 Mets hr did golf swing at a frequency of 30 times/min, and continued for 5 minutes in a mode of exercising for 1 min and then resting for 1 min. The maximal respiratory quotient of the male subject was measured with a cardio-pulmonary function tester from JAEGER Company of German during the exercising and it was 0.86. A contact pressure tester from AMI Company of Japan was used to measure the following maximal clothing pressures when wearing the elastic jacket in a motionless state: 0.57 kPa in a position between the elbow portion and the wrist portion,
0.33 kPa in the chest portion, and 0.39 kPa in the back side. The maximal clothing pressure in a motion state was 1.15
kPa at a position between the elbow portion and the wrist portion, 0.27 kPa in the chest portion, and 0.88 kPa in the back side. The colorfastness of the elastic jacket dyed with cationicdyeswas Class 4 or higher when measured according to JIS.

### Example 2:

Core-sheath composite deformation textured yarns made of 110 dtex /51 filament polyamide and 33 dtex polyurethane yarns were used in a proportion of 90 to 10 to produce a circular plain knit fabric with a gram weight of 180 g/m². A compression garment of size L using the knit fabric for 100% body circumference was finally made after the treatments of refining, dyeing, and forming. The circular knitted fabric was measured to have a maximal tightness
index of 0.7 and a maximal recovery stress of 1.1 N at 30∼80% elongation. A male subject having a body height of 173 cm, a body weight of 75 kg and monthly exercising at an amount of 86 Mets hr did jogging exercise at 8 km/hr for 20 min. The maximal respiratory quotient of the male subject was measured with a cardio-pulmonary function tester from JAEGER Company of German during the exercising and it was 1.02. A contact pressure tester from AMI Company of Japan was used to measure the following maximal clothing pressures when wearing the soft and elastic jacket in a
motionless state: 0.60 kPa at a position between the elbow position and the wrist portion, 0.31 kPa in the chest portion, and 0.36 kPa in the back side. The maximal clothing pressure in a motion state was 1.25 kPa at a position between the elbow portion and the wrist portion, 0.32 kPa in the chest portion, and 1.51 kPa in the back side. The color fastness of the soft and elastic jacket dyed with cationic dyes was Class 4 or higher when measured according to JIS.

### Example 3:

Core-sheath composite deformation textured yarns made of 140 dtex /70 filament PET fiber core and polyamide fiber sheath, and 33 dtex polyurethane yarns were used to in a proportion of 92 to 8 produce a circular plain knit fabric with a gram weight of 180 g/m². A compression garment of size L using the knit fabric for 80% body circumference was
finally made after the treatments of refining, dyeing, and forming. The circular knitted fabric was measured to have a maximal tightness index of 0.8 and a maximal recovery stress of 1.3 N at 30∼80% elongation. A female subject having a body height of 168 cm, a body weight of 60 kg and monthly exercising at an amount of 460 Mets·hr did upright push- ups exercise at a frequency of 30 times/min. The exercise mode was: Exercise: 1 min; rest: 1 min; Exercise: 2 min; rest: 1 min; Exercise: 3 min; rest: 1 min; Exercise: 4 min; rest: 1 min. The total time of the Exercise was 10 min. The maximal
respiratory quotient of the female subject was measured with a cardio-pulmonary function tester from JAEGER Company of German during the exercising and it was 1.02. A contact pressure tester from AMI Company of Japan was used to measure the following maximal clothing pressures when wearing the soft and elastic jacket in a motionless state: 0.60 kPa at a position between the elbow portion and the wrist portion, 0.33 kPa in the chest portion, and 0.39 kPa in the back side. The maximal clothing pressure in a motion state was 1.13 kPa at a position between the elbow portion and
the wrist portion, 0.43 kPa in the chest portion, and 1.68 kPa in the back side portion. The color fastness of the soft and elastic jacket dyed with cationic dyes was Class 4 or higher when measured according to JIS.

## Claims

1. A soft and elastic jacket being composed of an elastic weft knitted fabric, wherein the elastic weft knitted fabric comprises 5∼15% weight of elastic yarns and the rest of non-elastic yarns knitted with each other, wherein the elastic weft knitted fabric covers no less than 70 percent of the circumference of a body part of the soft and elastic jacket when the soft and elastic jacket is in a motionless state without being worn, characerized in that the elastic weft knitted fabric has a tightness index of not greater than 0.8 and a recovery stress of 0.3∼1.3 N at an elongation range of 30∼80%, wherein the tightness index is measured according to a method specified in JIS L-1096:1999, and the recovery stress is measured according to a method specified in JIS L-1096:1999.

2. The soft and elastic jacket according to claim 1 wherein the soft and elastic jacket has a clothing pressure of 0.6 kPa or less in a motionless state, and 2.5 kPa or less in a motion state, wherein the clothing pressure is measured by using a contact pressure tester in which the diameter of a bag as used is 20 mm.

3. The soft and elastic jacket according to claim 2 wherein the clothing pressure in a motionless state is 0.60 kPa or less at a portion between an elbow portion and a wrist portion, 0.33 kPa or less at a chest portion, and 0.40 kPa or less at a back side.

4. The soft and elastic jacket according to claim 2 wherein the clothing pressure in a motion state is 1.25 kPa or less at a portion between an elbow portion and a wrist portion, 0.45 kPa or less at a chest portion, and 1.85 kPa or less at a back side.

5. The soft and elastic jacket according to claim 1 wherein the elastic weft knitted fabric has a basis weight of 140-200 g/m².

6. The soft and elastic jacket according to claim 5 wherein the elastic yarns are polyurethane fibers.

7. The soft and elastic jacket according to claim 5 or 6 wherein the non-elastic yarns are modified polyethylene terephthalate fibers and/or polyamide fibers.

8. The soft and elastic jacket according to claim 7 wherein the non-elastic yarns are cationic dyeable PET fibers.

## Patentansprüche

1. Weiche und elastische Jacke, die aus einem elastischen Schussgewirk besteht, wobei das elastische Schussgewirk 5 bis 15 Gew.-% an elastischen Garnen und den Rest an miteinander verstrickten, nicht-elastischen Garnen aufweist,
- wobei das elastische Schussgewirk nicht weniger als 70 Prozent des Umfangs eines Körperteils der weichen und elastischen Jacke bedeckt, wenn sich die weiche und elastische Jacke in einem bewegungslosen Zustand befindet, ohne getragen zu werden, **dadurch gekennzeichnet, dass**
- das elastische Schussgewirk einen Dichtheitsindex von nicht mehr als 0,8 und eine Rückstellspannung von 0,3 bis 1,3 N bei einem Dehnungsbereich von 30 bis 80 % aufweist, wobei der Dichtheitsindex gemäß einem in JIS L-1096:1999 spezifizierten Verfahren und die Rückstellspannung gemäß einem in JIS L-1096:1999 spezifizierten Verfahren gemessen wird.

2. Weiche und elastische Jacke nach Anspruch 1, wobei die weiche und elastische Jacke einen Bekleidungsdruck von 0,6 kPa oder weniger in einem bewegungslosen Zustand und 2,5 kPa oder weniger in einem Bewegungszustand aufweist, wobei der Bekleidungsdruck unter Verwendung eines Kontaktdruckprüfers gemessen wird, bei dem Durchmesser eines verwendeten Beutels 20 mm beträgt.

3. Weiche und elastische Jacke nach Anspruch 2, wobei der Bekleidungsdruck in einem bewegungslosen Zustand 0,60 kPa oder weniger an einem Abschnitt zwischen einem Ellbogenabschnitt und einem Handgelenkabschnitt, 0,33 kPa oder weniger an einem Brustabschnitt und 0,40 kPa oder weniger an einer Rückseite beträgt.

4. Weiche und elastische Jacke nach Anspruch 2, wobei der Bekleidungsdruck in einem Bewegungszustand 1,25 kPa oder weniger an einem Abschnitt zwischen einem Ellbogenabschnitt und einem Handgelenkabschnitt, 0,45 kPa oder weniger an einem Brustabschnitt und 1,85 kPa oder weniger an einer Rückseite beträgt.

5. Weiche und elastische Jacke nach Anspruch 1, wobei das elastische Schussgewirk ein Basisgewicht von 140 bis 200 g/m² aufweist.

6. Weiche und elastische Jacke nach Anspruch 5, wobei die elastischen Garne Polyurethan-Fasern sind.

7. Weiche und elastische Jacke nach Anspruch 5 oder 6, wobei die nicht-elastischen Garne modifizierte Polyethylenterephthalat-Fasern und/oder Polyamid-Fasern sind.

8. Weiche und elastische Jacke nach Anspruch 7, wobei die nicht elastischen Garne kationisch färbbare PET-Fasern sind.

## Revendications

1. Veste souple et élastique qui est composée d'un tricot à mailles cueillies du type élastique, dans laquelle le tricot à mailles cueillies du type élastique comprend 5 à 15% en poids de fils élastiques et le reste étant des fils non élastiques tricotés les uns avec les autres, dans laquelle
le tricot à mailles cueillies du type élastique couvre au moins 70 pour cent de la circonférence d'une partie de corps de la veste souple et élastique lorsque la veste souple et élastique est dans un état de non-mouvement sans être portée, **caractérisée en ce que**
le tricot à mailles cueillies du type élastique a un indice de compacité non supérieur à 0,8 et un effort de recouvrance allant de 0,3 à 1,3 N à une plage d'allongement de 30 à 80%, dans laquelle l'indice de compacité est mesuré selon un procédé spécifié dans JIS L-1096:1999, et l'effort de recouvrance est mesuré selon un procédé spécifié dans JIS L-1096:1999.

2. Veste souple et élastique selon la revendication 1, dans laquelle la veste souple et élastique a une pression de vêtement inférieure ou égale à 0,6 kPa dans un état de non-mouvement, et inférieure ou égale à 2,5 kPa dans un état de mouvement, dans laquelle la pression de vêtement est mesurée en utilisant un testeur de pression de contact dans lequel le diamètre d'un sac tel qu'il est utilisé est de 20 mm.

3. Veste souple et élastique selon la revendication 2, dans laquelle la pression de vêtement dans un état de non-mouvement est inférieure ou égale à 0,60 kPa au niveau d'une partie entre une partie de coude et une partie de poignet, inférieure ou égale à 0,33 kPa au niveau d'une partie de poitrine et inférieure ou égale à 0,40 kPa au dos.

4. Veste souple et élastique selon la revendication 2, dans laquelle la pression de vêtement dans un état de mouvement est inférieure ou égale à 1,25 kPa au niveau d'une partie entre une partie de coude et une partie de poignet, inférieure ou égale à 0,45 kPa au niveau d'une partie de poitrine et inférieure ou égale à 1,85 kPa au dos.

5. Veste souple et élastique selon la revendication 1, dans laquelle le tricot à mailles cueillies du type élastique a une masse surfacique allant de 140 à 200 g/m2.

6. Veste souple et élastique selon la revendication 5, dans laquelle les fils élastiques sont des fibres de polyuréthane.

7. Veste souple et élastique selon la revendication 5 ou 6, dans laquelle les fils non élastiques sont des fibres de polyéthylène téréphtalate modifié et/ou des fibres de polyamide.

8. Veste souple et élastique selon la revendication 7, dans laquelle les fils non élastiques sont des fibres PET pouvant recevoir une teinture cationique.
